# EUROPEAN PATENT SPECIFICATION

(11) **EP 0 285 227 B1**
(45) Date of publication and mention of the grant of the patent: **25.11.1992**
(21) Application number: 88200608.3
(22) Date of filing: 31.03.1988
(51) Int. Cl.: D21H 17/26, D21H 23/50, B05D 1/02, B05B 13/02

(54) **A process for preserving paper sheets or webs and a device for carrying out that process**
Verfahren zur Konservierung von Bogen und Bahnen aus Papier und Vorrichtung zur Ausführung dieses Verfahrens
Procédé de conservation de feuilles de papier et dispositif pour la mise en oeuvre de ce procédé

(30) Priority: 01.04.1987 NL 8700766
(43) Date of publication of application: 05.10.1988
(73) Proprietor: B.V.B.A. Technische Handelsonderneming Jezet International, 2000 Antwerpen (BE)
(72) Inventor: De Leeuw, Guillaume Petrus Gerardus Marie, NL-4695 RD St.Maartensdijk (NL)
(74) Representative: Smulders, Theodorus A.H.J., Ir.

(56) References cited:
- DE-A- 2 112 997
- FR-A- 2 125 963
- US-A- 2 633 437
- US-A- 3 676 182
- US-A- 3 862 916
- US-A- 3 899 439
- US-A- 3 939 091
- US-A- 3 958 586
- ABSTRACT BULLETIN OF THE INSTITUTE OF PAPER CHEMISTRY, vol. 54, no. 7, January 1984, page 785, no. 7288, Appleton, Wisconsin, US; N.G. GERASIMOVA et al.: "Study of some aqueous sizes and sizing media used in restoration of paper"

## Description

This invention relates to a process for preserving archives and library materials in the form of paper sheets or webs and to a device suitable for use in carrying out that process.

US-A-3 676 182 discloses a process for treating e.g. paper sheets or webs throughout their thickness with a solution of a deacidification agent in an organic solvent or in a mixture of organic solvents and then drying same. The object of this known treatment is to neutralize the acid components contained in the paper and thereby to render the paper more resitant to prolonged storage in archives. Moreover, a polymeric strengthening agent for the paper can be included in the solution. The use of an organic liquid medium instead of an aqueous medium has the advantage that more rapid drying can be obtained while the time of contact with the printed matter present on the paper can be kept so short that this printed matter sustains no visible damage owing to the treatment conducted. The paper can be impregnated or sprayed with the solution and then be dried. Several techniques for applying the solution and also various methods of drying the treated product have been disclosed.

US-A-3 939 091 also discloses a liquid mixture on the basis of organic solvents designed for deacidifying paper. In this known mixture the empoyed agent effecting deacidification or, in other words, providing an alkaline component is methoxy magnesium methyl carbonate, called in this patent methyl magnesium carbonate.

US-A-3 862 916 discloses a composition for restoring and preserving papers. Said composition comprises a solution of a phenolic antioxidant and a polyvinyl acetal in an organic solvent mixture.

There has now been found a simple, efficient and inexpensive method of simultaneously deacidifying, strengthening, and at least partly drying archives and library materials in the form of paper sheets or webs.

Accordingly, this invention is characterized in that a solution of a deacidification agent and of a polymeric strengthening agent in a mixture of organic solvents comprising a mayor amount of methanol and a minor amount of acetone is sprayed onto one surface of the paper, and that a strong sucking action is exerted on the other surface of the paper so as to draw the solution through the entire thickness of the paper and also dry the treated paper at least partly.

As compared with the prior art, the process now claimed offers a number of important advantages: the solution can be more uniformly distributed throughout the thickness of the paper; the amount of solution can be more optimally dosed; and the process can be carried out more rapidly, partly because subsequent drying usually need not take place. The process claimed leads to an excellent total preservation of archives and library material which threatens to be lost forever without a timely appropriate treatment.

Suitable polymeric strengthening agents for use in the present solution are known per se adhesives for fibrous materials of cellulose or derivatives thereof. Suitable strengthening agents may be cellulose or starch ethers, such as hydroxyethyl cellulose and preferably hydroxypropyl cellulose. The latter product is sold by Hercules Powder Company under the name of Klucel L in the form of fine granules. The amount in which the strengthening agent is used is as a rule 5-40 g and preferably 5-30 g/l solution.

It is of essential importance that the polymeric strengthening agent be present in the solution in the dissolved state. This is in fact necessary to obtain a uniform distribution of the strengthening agent throughout the thickness of the paper to be treated. If the strengthening agent were not dissolved, it would only be deposited on and near the paper surface, so it would not be able to penetrate into the interior of the paper material so that more damage than advantage would be caused to the material to be preserved which is very vulnerable as it is. So when selecting the polymeric strengthening agent, but also when selecting the other constituents and their mutual ratios,one should always bear in mind that the final preserving liquid has to be a real solution.

Preferably, a suitable agent for preventing disintegration or decay of the polymeric strengthening agent is also dissolved in the treatment solution. Such agents may be bactericides and fungicides as well as agents for preventing enzymatic decomposition of the strengthening agent. Thymol is an example of a suitable agent preventing the development of bacteria and fungi in the case of using a cellulose ether as the polymeric strengthening agent. As a rule only a minor amount of such an agent is added against disintegration or decay.

Suitable examples of deacidification agents to be used in the present solution are to be found in US-A-3 676 182 and 3 939 091 discussed above. Preferably, inorganic deacidification agents are used, and the following compounds may be mentioned as examples thereof: magnesium methoxide, magnesium methyl carbonate, magnesium ethyl carbonate, methoxy magnesium methyl carbonate, and ethoxy magnesium ethyl carbonate. In particular, methoxy magnesium methyl carbonate has proved to be eminently suitable. The deacidification agent is usually employed in an amount of 0.7-2.5 g and preferably of 1.0-2.0 g/l solution. Such a concentration is sufficient to adjust the pH of the paper to a value of 8-8.5 and further to provide a sufficient additional amount to ensure a prolonged buffer effect at that pH. A number of the above-mentioned inorganic deacidification agents is commercially available, usually in the form of a solution in a lower alcohol or in a mixture of a lower alcohol and a chlorofluorohydrocarbon.

The selection of a suitable mixture of organic solvents is very important, since, as stated before, all the components of the preserving liquid must dissolve therein. A mixture of a major amount of methanol and a minor amount of acetone has proved to be very suitable and is used according to the invention, especially a mixture of methanol and acetone in a volume ratio of about 4/1.

The present preserving liquid can be easily prepared by combining the different components in the appropriate amounts and, if required, stirring same with moderate heating until the solids have dissolved. The deacidification agent is then mostly added in the form of a concentrated solution in an organic solvent. If necessary, the resulting solution may be filtered to remove all the undissolved residues. The preserving liquid may also be prepared in the form of a concentrate diluted for use as far as necessary. Both the concentrate and the ready-for-use preserving liquid are very stable and can be stored for extended periods of time.

A formulation of a ready-for-use preserving liquid with which excellent results have been obtained has the following composition:

| | |
|---|---|
| - methanol | 78 vol.% |
| - acetone | 20 vol.% |
| - methoxy magnesium methyl carbonate (0.5 M in methanol) | 2 vol.% |
| - Klucel L (hydroxypropyl cellulose from Hercules Powder Co.) | 2 wt.% |
| - thymol | 0.2 wt.% |

The preserving liquid is applied by spraying to one surface of the paper sheet or web and a strong sucking action is exerted on the other surface of the paper. Preferably, the paper is supported by a carrier allowing the passage of liquid, and the liquid is sprayed onto the free paper surface while a strong sucking action is exerted through the supporting carrier so that the paper is uniformly impregnated with the liquid throughout its thickness and is also at least partly dried. If necessary, further drying can be effected by suction drying for an extended period of time or by using any mild drying technique, e.g., with a hot air stream. The amount of preserving liquid to be applied depends on different factors, such as the nature, condition and thickness of the paper. On the average, however, it has turned out that excellent preservation is obtainable with an amount of preserving liquid of 0.2-0.5 g/dm² paper area.

This invention also relates to a device for carrying out the above described preservation of paper sheets or webs. This device is characterized in that it contains a treatment chamber provided in the lower part with a paper feed opening in one end wall and with a paper discharge opening in the opposite end wall, with a suction receptacle being arranged between the feed and discharge openings and comprising at the top a large number of perforations, there being provided a conveyor belt allowing the passage of liquid, which conveyor belt is capable of moving around the suction receptacle and is positioned against the top thereof, said conveyor belt being provided with five openings which are larger at the side facing the top of the suction receptacle than at the side for conveying paper, at least one liquid sprayer which is automatically adjustable being present in the upper part of the treatment chamber near the feed opening.

The treatment chamber proper may be composed of aluminum sections with aluminum sheeting and with one side wall in the direction of transport consisting of a transparent material, such as a polycarbonate sheet, so that the progress of the treatment may be monitored.

The treatment chamber may be placed as a superstructure ton a substructure, and the latter can be utilized to accommodate the operating and auxiliary mechanisms, such as an electronic and pneumatic control unit, a storage tank for the preserving liquid, a pressure bottle containing propellent gas (e.g., CO₂), a compressor, an exhaust fan, a motor, the required conduits and connecting pieces etc.

A slot for inserting the paper to be treated is provided at the feed end of the treatment chamber. When paper is inserted, a sensor which may be provided near that feed end will transmit a signal which causes the liquid sprayer(s) to function. When paper is no longer inserted, the sensor in question can stop the spraying of liquid by means of a signal.

Also provided near the feed opening may be sensors recording the thickness, nature and/or sizes of the paper inserted and transmitting, as a function thereof, signals controlling the speed of the conveyor belt, the amount of spray liquid and/or the area of the surface to be sprayed.

Through the feed slot the paper comes to rest on a conveyor belt which is capable of moving around a suction receptacle in the lower part of the treatment chamber and is positioned against the perforated top of the suction receptacle.

Provided in the upper part of the treatment chamber, near the feed opening, is at least one automatically adjustable liquid sprayer for atomizing the preserving liquid in the direction of the conveyor belt. As a rule, two liquid sprayers are present, and preferably, both the height and the width of the liquid sprayer(s) are adjustable so as to exactly control the area to be sprayed. This can be effected automatically by means of a sensor near the feed opening, as stated before.

The suction receptacle is provided, e.g., in a side wall in the direction of transport, with a plurality of suction nozzles, e.g., three, which ensure a proper suction and exhaustion during the entire transport throughout suction and exhaustion during the entire transport through the treatment chamber. The preserving liquid is thereby uniformly distributed throughout the thickness of the paper to be treated, and the paper is also at least partly and usually even completely dried. This can be carried out by a skilled worker in a rather simple and precise way. The exhausted vapours can be collected and processed further.

The conveyor belt may be a woven endless belt and it is of the self-discharging type, which means that the fine openings present in the direction of thickness of that belt are larger at the side facing the top of the suction receptacle than at the side for conveying paper, which prevents that belt from becoming easily clogged owing to solids from the preserving liquid sucked in.

The size of the treatment chamber in the direction of transport is preferably selected so that the distance to be traversed is sufficient to dry the treated paper. If required, however, the part of the treatment chamber closer to the discharge opening may comprise means for carrying out an additional thermal drying treatment. Such means may be means for effecting a hot air stream or infrared radiation.

Finally, the treatment chamber is provided with a discharge slot at the end of the conveyor belt. The treated paper discharged through that slot can be collected in a collecting receptacle.

## Claims

1. A process for preserving archives and library materials in the form of paper sheets or webs by treating same with a solution of a deacidification agent and of a polymeric strengthening agent for the paper in a mixture of organic solvents, characterized in that a solution of said agents in a mixture of organic solvents comprising a major amount of methanol and a minor amount of acetone is sprayed onto one surface of the paper, and that a strong suction action is exerted on the other surface of the paper so as to draw the solution through the entire thickness of the paper and also dry the treated paper at least partly.

2. A device suitable for use in preserving paper sheets or webs according to the process of claim 1, said device comprising a treatment chamber and at least one liquid sprayer, characterized in that
- the treatment chamber is provided in the lower part with a paper feed opening in one end wall and with a paper discharge opening in the opposite end wall,
- a suction receptable is arranged between the feed and discharge openings said suction receptacle comprising at the top a large number of perforations, there being provided a conveyor belt allowing the passage of liquid, which conveyor belt is capable of moving around the suction receptacle and is positioned against the top thereof, said conveyor belt being provided with fine openings which are larger at the side facing the top of the suction receptable than at the side for conveying paper,
- at least one liquid sprayer which is automatically adjustable is present in the upper part of the treatment chamber near the feed opening, and
- means for carrying out an additional thermal drying can preferably be provided in the part of the treatment chamber which is closer to the discharge opening.

## Patentansprüche

1. Verfahren zur Konservierung von Archiven und Bibliothekmaterialien in Form von Bogen und Bahnen aus Papier durch Behandeln derselben mit einer Lösung aus einem Entsäurungsmittel und einem polymeren Festigungsmittel für Papier in einem Gemisch aus organischen Lösungsmitteln,
**dadurch gekennzeichnet,**
daß eine Lösung dieser Mittel in einem Gemisch aus organischen Lösungsmitteln, welches einen größeren Anteil Methanol und einen kleineren Anteil Aceton enthält, auf eine Oberfläche des Papiers aufgesprüht wird und daß eine starke Saugwirkung auf die andere Oberfläche des Papiers ausgeübt wird, um die Lösung durch die gesamte Dicke des Papiers hindurchzuziehen und außerdem das behandelte Papier wenigstens teilweise zu trocknen.

2. Vorrichtung zur Konserviervung von Bogen oder Bahnen aus Papier gemäß dem Verfahren aus Anspruch 1, wobei die Vorrichtung eine Behandlungskammer und wenigstens einen Flüssigkeitssprüher aufweist,
**dadurch gekennzeichnet,**
daß
- die Behandlungskammer im unteren Teil mit einer Papierzufuhöffnung in einer Stirnwand und mit einer Papierauslaßöffnung in der gegenüberliegenden Stirnwand versehen ist,
- ein Sauggefäß zwischen der Zufuhr- und der Auslaßöffnung vorgesehen ist, welches am oberen Ende eine große Anzahl von Perforationen aufweist, wobei ein Transportband vorgesehen ist, das den Durchtritt von Flüssigkeit gestattet, wobei dieses Transportband um das Sauggefäß herum bewegt werden kann und gegen das obere Ende desselben positioniert ist, wobei das Transportband mit feinen Öffnungen versehen ist, die an der Seite, welche dem oberen Ende des Sauggefäßes zugewandt ist, größer sind als an der zum Transport von Papier vorgesehenen Seite,
- wenigstens ein Flüssigkeitssprüher, der automatisch einstellbar ist, im oberen Teil der Behandlungskammer, nahe der Zufuhröffnung vorgesehen ist, und
- Einrichtungen zum Ausführen einer zusätzlichen thermischen Trocknung in dem Teil der Behandlungskammer, welcher sich näher der Auslaßöffnung befindet, vorzugsweise vorgesehen sein können.

## Revendications

1. Procédé de conservation des archives et du matériel de bibliothèque sous forme de feuilles ou de bandes de papier, consistant à traiter celles-ci avec une solution constituée d'un agent de dé-acidification et d'un agent polymère de renforcement du papier, dans un mélange de solvants organiques, caractérisé en ce que la solution desdits agents dans un mélange de solvants organiques comprenant une proportion majoritaire de méthanol et une proportion minoritaire d'acétone est diffusée sur l'une des surfaces du papier, et qu'une action de succion violente est exercée sur l'autre surface du papier de façon à aspirer la solution à travers l'entière épaisseur du papier et aussi en ce que le papier traité est séché au moins partiellement.

2. Appareil destiné à être utilisé dans le procédé de conservation des bandes ou des feuilles de papier selon la revendication 1, ledit appareil comprenant une chambre de traitement et au moins un diffuseur de liquide caractérisé en ce que:
- la chambre de traitement est munie, dans sa partie inférieure, d'une ouverture d'alimentation du papier située à une paroi d'extrémité, et d'une ouverture d'éjection du papier située à l'autre paroi d'extrémité;
- un réceptacle de succion est disposé entre lesdites ouvertures d'alimentation et d'éjection, ledit réceptacle de succion comprenant sur sa partie supérieure un grand nombre de perforations, ledit réceptable comprenant une bande convoyeuse perméable, ladite bande convoyeuse étant susceptible de se déplacer autour dudit réceptacle de succion, et étant disposée contre la partie supérieure de ce réceptacle, ladite bande convoyeuse étant munie de petites ouvertures qui sont plus grandes du côté faisant face à la partie supérieure du réceptacle de succion que du côté de convoyage de papier;
- au moins un diffuseur de liquide automatiquement ajustable est présent, dans la partie supérieure de la chambre de traitement, au voisinage de l'ouverture d'alimentation; et
- des moyens pour effectuer un traitement additionnel de séchage thermique, peuvent être disposés de préférence dans la partie de la chambre de traitement qui est la plus voisine de l'ouverture d'éjection.
